

1

3,743,531

PHOTOGRAPHIC PRODUCT

Gerald Louis Ducharme, Rochester, N.Y., assignor to  
Eastman Kodak Company, Rochester, N.Y.  
No Drawing. Filed July 19, 1971, Ser. No. 164,050  
Int. Cl. B41m 1/18; C23c; D21K

U.S. Cl. 117—76 P

16 Claims

ABSTRACT OF THE DISCLOSURE

Photographic elements comprise a support having thereon, a layer containing barium sulfate, polyvinyl alcohol and an optical brightener such as a stilbene, anthracene, terphenyl, tetraphenylbutadiene or quinoxaline. Particularly useful brighteners are stilbene brighteners. The support can be comprised of paper or paper having the baryta layer overcoated with polyolefin coating such as polyethylene. These elements can be used as supports for receiving layers for use in the chemical transfer system and also as a support for silver halide emulsions or similar light sensitive coatings.

FIELD OF INVENTION

This invention relates to novel photographic elements. More particularly, this invention relates to photographic supports having a stable brightened barium sulfate layer thereon in order to provide improved supports for photographic prints and to a coating composition comprising a stable brightening agent.

BACKGROUND OF THE INVENTION

The highlight areas of photographic color prints and other products, such as, fibrous or plastic articles are often made to look whiter by incorporating optical brightening agents. These brightening agents fluoresce under radiation with ultraviolet light, emitting visible light, usually bluish in hue thus enhancing the whiteness of the object. Such products also frequently contain ultraviolet sensitive ingredients such as dyes, organic polymers, etc., which require protection from irradiation in the ultraviolet re-



gion, especially from 360-400 m $\mu$ . Brighteners are inherently ultraviolet absorbers and depend on this characteristic for the energy required to fluoresce in the visible region of the spectrum. Most of the known brightening agents are decomposed by prolonged exposure to ultraviolet radiation, and thus lose their ability to fluoresce and serve as brightening agents. Brighteners containing substituted vinylene groups, e.g., stilbenes, styrenes and vinylenes are well known and are efficient brighteners which absorb and fluoresce in desirable regions of the spectrum. Other known brighteners include those that contain at least one heterocyclic five-membered or six-membered ring, for example, an oxazole, a thiazole, an imidazole, a triazole, a pyrazole, a furan, a thiophene, or a coumarin ring.

Photographic paper conventionally has a layer thereon containing barium sulfate known as baryta or blanc fixed in a colloid binder such as gelatin. The paper can have a layer of gelatin or similar colloid coated over the baryta layer containing a silver precipitating agent such as noble metal nuclei for use in a diffusion transfer process. The

2

brightener can be incorporated in the baryta layer under the layer containing the image.

It has been particularly desirable to incorporate a water soluble brightener in the baryta layer since this provides a relatively easy method of providing a coating and avoids the problem of dispersing a water insoluble material in a hydrophilic colloid containing a barium sulfate pigment. A coating of this type is described in U.S. Pat. 3,269,840, issued to Pattyn et al. Aug. 30, 1966, in which a baryta layer is provided which employs gelatin as the essential binding agent and has incorporated in the coating a water-soluble brightener and a water-soluble vinylpolymer, in order to avoid the problem of rinsing or bleeding of the brightening agents out of the layers to which they are added. However, the problem of stability of the brightener in the baryta layer remains. Therefore, it has been desirable to provide a baryta layer containing a water soluble brightening agent which would be more stable and which would also be essentially free from leaching or bleeding from the layer.

One object of this invention is to provide a coating comprising baryta, an optical brightener and polyvinyl alcohol which when coated on a support has improved fading resistance to light, humidity and temperature. Another object of this invention is to provide a baryta layer which can be overcoated with a relatively clear polymeric layer which can be used to provide an improved photographic print. A further object is to provide a brightened photographic print. A still further object is to provide a stable brightened photographic print produced by a diffusion transfer process.

SUMMARY OF THE INVENTION

It has now been found that the above objects are attained by preparing a coating composition by dispersing the baryta and brightener in polyvinyl alcohol as a binder substantially free from a protein such as gelatin. In a preferred embodiment, a paper base is employed which has coated thereon a baryta formulation containing polyvinyl alcohol and a brightener having the following chemical structure:



In still another preferred embodiment, the baryta layer is overcoated with a layer of polyethylene and the resulting element used as a receiving sheet in a diffusion transfer process. A product having a brightened baryta layer of this invention with a polyethylene overcoat can also be used as a photographic support by coating thereon a light-sensitive coating such as a silver halide emulsion.

A receiving element as described above is used advantageously to provide a photographic print having an image in a receiving layer on a support by the photographic silver salt diffusion transfer process or color diffusion transfer process.

DESCRIPTION OF THE PREFERRED EMBODIMENTS

Any suitable support may be used on which to place the baryta layer containing polyvinyl alcohol and brightener. However, paper is our preferred support although it will be understood that supports including polymeric materials such as polyesters, cellulose esters, and the like, glass, metal, etc., may all be used.

Suitable paper supports include any of the conventional paper supports including those prepared from cotton, linen, and wood (sulfate and sulfite pulped). Such supports are typically about 5-60 pounds per 1,000 square foot. A particularly desirable paper base is that having a high alpha cellulose content. Advantageously the paper base can have wet strength imparted by the incorporation of wet strength resin. If the coating to be applied is not adversely effected by formaldehyde, the wet strength resin can be for example melamine formaldehyde or urea formaldehyde resin. However, where a coating such as a photographic emulsion adversely effected by formaldehyde is used, it is desirable to incorporate a non-aldehydic wet strength resin in the paper, for example, a cationic thermosetting polyamide-epichlorohydrin resin as described in U.S. Pat. 2,926,154, available commercially under the name "Kymene".

The polyvinyl alcohol is substantially completely deacetylated polyvinyl acetate containing at least about 98% polyvinyl alcohol.

In addition to the barium sulfate dispersed in the polyvinyl alcohol coating, there may also be present a blue pigment or dye or a mixture of blue pigment and magenta pigment, which further improves the quality of the photographic prints obtained. The amount of tint or colored pigment when used is kept minor ordinarily being no more than 1% by weight based on the coating composition, preferably a fraction of 1%. The pigments used should be non-wandering and compatible with a silver halide photographic emulsion so as not to effect the sensitivity of the emulsion and should not wander from the baryta layer either to the emulsion layer or to the support. Also these pigments should be light stable and if an extrusion polymeric coating is used, the brightened layer should exhibit light and heat stability.

Some pigments which are examples of pigments of this type which are useful in barium sulfate-polyvinyl alcohol coatings in accordance with the invention are:

#### BLUE PIGMENTS

##### Ultra-Marine Blue EBEX

Manufacturer: Ultramarine Chemical Co.  
Composition:

Silicon dioxide  
Aluminum oxide  
Sodium oxide  
Sulfur

Description:

Vendor No. 59-3805.  
Pigment Blue 29 Color Index 77007.

Shepard Cobalt Blue #3

Manufacturer: Shepard Co.

Composition: Stoichiometric mixture of cobalt oxide and aluminum hydrate.

Description: Pigment Blue 28.

Cobalt Aluminated Blue V-3285

Manufacturer: Ferro Colors Corp.

Composition: Mixture of cobalt oxide and aluminum oxide.

Fastusol Blue Dye LFFRL

Manufacturer: General Aniline and Film  
E.I. Direct Blue #108 Color Index 51320

#### MAGENTA PIGMENTS

Raspberry V-6260 or Raspberry V-8295

Manufacturer: Fero Colors Corp.

Composition: Mixture of cobalt oxide and phosphorus oxide.

Hostaperm Pink E-13-7000

Manufacturer: American-Hoechst Co.

Composition: Quinacridone Type Red.

Description: Pigment Red-122.

In a typical coating composition the blue dye or pigment can comprise from about 0.001 to about 0.010%, by weight, of the baryta coating composition and the magenta pigment can comprise from about 0.1 to about 1.0%, by weight, of the baryta coating composition.

The barium sulfate may be naturally occurring or synthetic. Synthetic barium sulfate, sometimes known as blanc fixe, is typically prepared by the action of barium chloride on aluminum sulfate. The average particle size is generally below about 1.5 microns and preferably between about 0.25 and 1.0 micron.

Barium sulfate may be coated in an amount of about 2.5 to about 6.0 grams per square foot and polyvinyl alcohol about 5 to 20% by weight of the baryta layer.

The term "optical brightening agent" as used herein is intended to include those colorless or substantially colorless organic compounds which absorb ultraviolet light from sunlight or fluorescent light and emit the absorbed energy as visible blue or blue-green light. Thus, such compounds contain fluorescent chromophores in contradistinction to dyes, which contain colored chromophores. Water soluble indicates a solubility of at least 1 part in 10 parts of water at 20° C.

Suitable optical brightening agents include, for example, those brighteners selected from the following general classes of organic compounds: triazine-stilbenes, coumarins, anthracenes, terphenyls, tetraphenylbutadienes, quinoxalines, and the like. Triazine stilbene compounds which are conventional for use as fluorescent agents and as optical brightening agents, are described in U.S. Pat. 2,933,390 and have the following general formula:



wherein R<sub>6</sub>, R<sub>7</sub>, R<sub>2</sub>, and R<sub>3</sub> each represent a hydrogen atom, hydroxyl, aryloxy (e.g., phenoxy, o-toloxyl, p-sulfoxy, etc.), alkoxy (e.g., methoxy, ethoxy, etc.) a halogen atom (e.g., chlorine, bromine, etc.), a heterocyclic radical (e.g., morpholinyl, piperidyl, etc.), an alkylthio group (e.g., methylthio, ethylthio, etc.), an arylthio group (e.g., phenylthio, tolylthio, etc.), a heterocyclithio group (e.g., benzothiazylthio, etc.), an amino group, an alkylamino group (e.g., methylamino, ethylamino, propylamino, dimethylamino, diethylamino, decylamino, cyclohexylamino,  $\beta$ -hydroxyethylamino,  $\beta$ -hydroxyethylamino,  $\beta$ -sulfoethylamino, etc.), an arylamino group (e.g., anilino, o-, m-, and p-sulfoanilino, o-, m-, and p-chloroanilino, o-, m-, and p-carboxyanilino, hydroxyanilino, sulfonaphthylamino, o-, m-, and p-aminanilino, p-acetamidoanilino, etc.), etc., and R<sub>4</sub> and R<sub>5</sub> each represent a hydrogen atom or a water-solubilizing group, such as sulfo, carboxyl, etc. (as well as alkali metal or amine salts of such groups).

Examples of these compounds include 4,4'-bis[4-(3-sulfoanilino)-6-amino-s-triazin-2-ylamino]-stilbene-2,2'-disulfonic acid; 4,4'-bis[4,6-di( $\beta$ -hydroxyethylamino)-s-triazin-2-ylamino]-stilbene-2,2'-disulfonic acid, and the like.

Compounds of the above type are also described in one or more of the following patents: U.S. 2,171,427; 2,473,475; 2,595,030; 2,660,578; British Pats. 595,065; 623,849; 624,051; 624,052; 678,291; 681,642; 705,406. Additionally, compounds suitable for use in the reception element of the present invention are commercially available under such trade names as Tinopa [SP, WR, SFG, BV277, 2B, GS, NG], Leucophor B. Calcophor White MR, Blancofor SC, Hitamine [BSP, N, Sol., 6T6], and the like.

75 Suitable coumarin optical brightening agents are, for

example, the 3-phenyl-7-ureidocoumarins described in British Pat. 786,234 and which have the general formula:



wherein R<sub>1</sub> represents NH<sub>2</sub> or an organic primary or secondary amine, such as, for example, methylamino, diethylamino, etc., and R<sub>2</sub> represents a phenyl group, such as, for example, phenylthio, anilino, etc. or a halogen.

Examples of these compounds include: N<sup>1</sup>-[3-p-methyl phenyl-coumarinyl-(7)]-urea; N-propyl-N<sup>1</sup>-[3-phenyl-coumarinyl - (7)]urea; N-3-sulphoethyl-N<sup>1</sup>-3-phenyl coumarinyl-(7)-urea and the like. These compounds are commercially available under such trade names as Tinopal SFG (Geigy), etc.

Similarly, anthracenes, terphenyls, tetraphenylbutadienes and quinoxalines are conventional optical brightening agents and are well known in the art. Preferably the brightener is water soluble.

The concentration of the optical brightening agent may be varied over a wide range. Suitable concentrations include those in the range of between about 0.25 and about 10 milligrams of the optical brightening agent per square foot of reception element surface area, preferably between about 1.0 and about 5.0 milligrams per square foot. Higher concentrations of the brightening agent may be employed, but it is both unnecessary and impractical to do so.

The brightening compositions of this invention are advantageously used in image-receiving elements that are used to receive diffusion transfer images during the diffusion transfer process. In these processes, a light-sensitive diffusion transfer element containing a light-image exposed silver halide emulsion is processed with the exposed emulsion layer in contact with the silver precipitating layer of an image-receiving element in the presence of a silver halide developing agent, such as hydroquinone, 1-phenyl - 3 - pyrazolidone, p-methylaminophenol, etc., a silver halide solvent or complexing agent, such as an alkali metal thiosulfate, ammonium thiosulfate, an alkali metal thiocyanate, ammonium thiocyanate, etc. In a particularly useful process, a thickening agent, such as carboxymethylcellulose, carboxyethylcellulose, etc. is used.

During development, undeveloped silver halide forms a complex with the complexing agent which diffuses in an imagewise manner to the silver-precipitating layer on the image-receiving element where a silver image is precipitated from the silver halide complex. In an integral element, a silver halide emulsion coated over a silver precipitating layer is removed such as by washing, to disclose the transferred image.

In a color diffusion transfer process, an image-exposed light-sensitive silver halide color diffusion transfer element is contacted with the receiving layer of an image-receiving element in the presence of a developer solution which causes the release of a diffusible dye image that transfers to the mordanted receiving layer. The desired dye image remains in the receiving layer when the receiving element is separated from the developed diffusion transfer element. The diffusible dye image is formed from an incorporated non-diffusible coupler that couples with an imagewise pattern of oxidized primary aromatic amine color developing agent, produced by development of light-exposed silver halide. In another system, the dye image is formed from incorporated dye developing agents, such as hydroquinone derivatives that contain a chromophore as a substituent; the hydroquinone form of these compounds forms in the alkaline developer solution a diffusible dye while the dye developer that is oxidized to the quinone form (when it develops light-exposed silver halide to silver) is insoluble and does not diffuse to the image-receiving layer.

The image-receiving elements of this invention usually comprise a support as described previously that has been coated in succession with (1) a baryta layer containing the brightening composition, and (2) an image-receiving layer for a silver image comprising a silver precipitating agent or an image-receiving layer for a dye image comprising any suitable hydrophilic colloids containing a basic mordant for mordanting acid solubilized diffusible dyes.

Usually it is advantageous to have a hydrophobic resin layer between the baryta layer and the image-receiving layer. Hydrophobic resins that are advantageously used include poly(ethylene terephthalate), polyethylene, polypropylene, poly(3-methylbutene-1), poly(octene-1), poly-decene-1), polyamides, polyacetate, polycarbonates, cellulose triacetate, cellulose acetate butyrate, ethyl cellulose, etc.; preferably the hydrophobic resin layer is treated with corona discharge techniques just prior to coating the first hydrophilic colloid layer over the resin as described in U.S. patents such as 3,220,842, 2,864,755, 2,864,756, etc.

Any suitable silver precipitant is advantageously used in the receiving layer. As examples of suitable silver precipitating agents and of image-receiving elements containing such silver precipitating agents, reference may be made to U.S. Pat. Nos. 2,698,237, 2,698,238 and 2,698,245, issued to Edwin H. Land on Dec. 28, 1954; U.S. Pat. No. 2,774,667, issued to Edwin H. Land and Meroe M. Morse on Dec. 18, 1956, U.S. Pat. No. 2,823,122, issued to Edwin H. Land on Feb. 11, 1958, U.S. Pat. No. 3,396,018, issued to Beavers et al., Aug. 6, 1968 and also U.S. Pat. 3,369,901, issued to Fogg et al., Feb. 20, 1968. The noble metals, silver, gold, platinum, palladium, etc. in the colloidal form are particularly useful.

Noble metal nuclei are particularly active and useful when formed by reducing a noble metal salt using a borohydride or hypophosphite in the presence of a colloid. The metal nuclei are prepared in the presence of a colloid such as gelatin and coated on the receiving element. The coating composition generally contains not only nuclei, but also reaction products which are obtained from reducing the metal salt.

The amount of colloid used in preparing the above active noble metal nuclei can be varied depending upon the particular colloid, reducing agent, ratio of proportions, etc. Typically, about 0.5% to about 20%, by weight, based on the total reaction mixture of colloid is used, preferably from about 1% to about 10%.

In a particularly useful embodiment, 30 to 80  $\mu\text{g./ft.}^2$  of the active noble metal nuclei in 80 mg. of colloid (solids basis) is coated per square foot of support. The colloid binder is advantageously coated in a range of about 5 to about 50  $\mu\text{g./ft.}^2$ . Suitable concentrations on the receiving sheets of active noble metal nuclei as disclosed above can be about 1 to about 200  $\mu\text{g./ft.}^2$ . Other silver precipitants can be coated in a concentration of up to 5  $\mu\text{g./ft.}^2$ .

Any mordants that have a charge opposite to the charge of the dye being transferred are used to advantage in the image-receiving elements of my invention for dye transfer images. Since most of the useful photographic image-transfer dyes have acidic solubilizing groups, basic or cationic mordants are generally used. Typical mordants are organic quaternary phosphonium salts, organic tertiary sulfonium salts and organic quaternary ammonium salts. Suitable mordants include polymers of amino guanine derivatives of vinyl methyl ketone described in Minsk, U.S. Pat. 2,882,156. Other suitable mordants include the 2-vinyl pyridine polymer metho-p-toluene sulfonate, poly 4-vinyl-pyridine, thorium salt and similar compounds described in Sprague et al., U.S. Pat. 2,484,430.

A particularly useful class of mordanting compositions is disclosed in Bush, U.S. Pat. 3,271,147. Basic or cationic, nonpolymeric mordant compounds of Bush include quaternary ammonium and phosphonium, and tertiary sulfonic composition in which there is linked to the N, P or S

onium atom at least one hydrophobic ballast group, such as long-chain alkyl or substituted alkyl groups. The onium atom can be part of an open-chain or of a heterocyclic ring and there can be more than one onium ring in the molecule. When referring to the nonpolymeric nature of the mordant compounds of such mordanting compositions, it is understood that the cationic or the basic mordant does not have regularly occurring units containing the cationic group beyond the dimer structures. However, the ballast group attached to the quaternary or ternary atom 10 of the cation group can contain repeating groups such as tetraethoxy, polymethylene, etc.

In both the black and white and color diffusion transfer processes it is useful to have a polymeric acid layer located under the image receiving layer as described in 15 Rogers et al. U.S. Pat. No. 3,353,956 issued Nov. 21, 1967 to act as an alkali scavenging layer. Additional materials which may be used include a copolymer of acrylic acid and a monomer containing an active methylene function that serves as a site for cross-linking with conventional hardening agents such as aldehydes or vinyl sulfones. Typical polymers are disclosed in Smith U.S. Pat. 3,488,708 issued Jan. 6, 1970. Particularly useful copolymers are copoly (acrylic acid/2-acetoacetoxyethyl methacrylate) containing 90 wt. percent or 95 wt. percent 20 acrylic acid and copoly (acrylic acid/N-cyananoacetyl-N-methacryloylhydrazine) containing 90 wt. percent or 95 wt. percent acrylic acid.

The following examples are included for further understanding of the invention:

#### EXAMPLE 1

A paper base is coated at a coverage of 55 gms./m.<sup>2</sup> (dry) with the following composition:

|                         | Dry weight, gms. |
|-------------------------|------------------|
| Fastusol Blue Dye       | .04              |
| Raspberry V8295 Pigment | 4.32             |
| Blanc Fixe              | 800.00           |
| Dispersing agent        | 2.50             |
| Polyvinyl alcohol       | 106.00           |
| Uvitex CF*              | 12.00            |
| 2,3-dihydroxy-dioxane   | 12.00            |
| Spreading agent         | 0.60             |
| Colloidal silica        | 5.40             |
| Total                   | 942.86           |

\*Uvitex CF.



Samples of the coated base are exposed to full spectrum lighting at 1800 foot candle intensity, under conditions of 85% RH and 110° F. After six days exposure there is very little evidence of fluorescent fading or color change. Similar systems using gelatin instead of polyvinyl alcohol as a binder show a distinct loss of fluorescence and color shift when exposed to the same conditions of light, humidity and heat.

#### EXAMPLE 2

Baryta coated paper samples are prepared as described in Example 1. Both the sample employing polyvinyl alcohol as a binder and the sample employing gelatin are

5 overcoated with a substantially clear layer of polyethylene and used as support for a photographic silver chloride emulsion. After processing to obtain a silver image on the support, the samples are exposed as in Example 1 to 1800 foot candle intensity, of light at 85% RH and 110° F., with the same resistance to fading for the polyvinyl alcohol sample as compared to a distinct fading of brightener fluorescence in the sample using gelatin.

#### EXAMPLE 3

Paper samples are prepared as described in Example 1. In addition, pigmented polyethylene is coated on the back side of the paper and clear polyethylene over the brightened baryta layers. Over the brightened baryta layer and the polyethylene surface, after electron bombardment, is coated a layer of cellulose acetate containing copoly (styrene/maleic anhydride) and over this layer a gelatin layer containing silver precipitating nuclei. In another embodiment for use in color diffusion transfer, a gelatin mordanted receiving layer is used instead of a silver precipitating layer. When the receiving sheets described are used in black and white and in color diffusion transfer systems respectively, they are found to provide photographic prints having good characteristics. The gelatin dispersion of the brightener is found to fade as compared to the polyvinyl alcohol sample which is stable to fading under the conditions described in Example 1.

#### EXAMPLE 4

30 A brightened baryta layer containing polyvinyl alcohol on paper is used as a support and coated in succession (over the brightening layer) with (1) an ordinary blue-sensitive gelatin silver chlorobromide emulsion and a dispersion of a yellow dye-forming coupler of the type described in McCrossen et al. U.S. Pat. 2,875,057 (2) a gelatin interlayer, (3) a gelatin layer containing an ordinary green-sensitized gelatin silver chlorobromide emulsion, a dispersion of a magenta dye-forming coupler, such as, one of the couplers described in Loria, et al. U.S. Pat. 2,600,788, (4) a gelatin layer, (5) a gelatin layer containing an ordinary red-sensitized gelatin silver chlorobromide emulsion, a dispersion of a cyan dye-forming coupler such as is described in Fierke U.S. Pat. 2,801,171, and (6) a gelatin protective layer.

40 The photographic element is exposed in an intensity scale sensitometer and then color processed as described in Example 1, columns 5 and 6 of Van Campen U.S. Pat.

65 2,956,879 using 12 minutes development in the color developer. The processed color print has brightened highlights that even after prolonged exposure to the light, retain their brightness to a much higher degree than control color prints made by the same way except that the brightening agent is dispersed in gelatin.

#### EXAMPLE 5

70 The brighteners listed below are coated in clear layers of polyvinyl alcohol and gelatin at concentrations of 1.0% of the dry polyvinyl alcohol or gelatin. The layers are coated at a coverage of approximately 10 gm./m.<sup>2</sup> on a clear polyethylene coated support.

| Brightener               | Manu-facturer | Binder       | Fresh                     | 2 days<br>fluorescence<br>1,800 ft. cd. | 6 days                    |
|--------------------------|---------------|--------------|---------------------------|-----------------------------------------|---------------------------|
| 1..... Tinopal 4BM.....  | Geigy.....    | (PVA<br>Gel) | Excellent.....<br>do..... | Excellent.....<br>Good.....             | Excellent.....<br>NG..... |
| 2..... Tinopal RBS.....  | do.....       | (PVA<br>Gel) | do.....                   | Excellent.....<br>NG.....               | Good.....<br>NG.....      |
| 3..... Tinopal AMS.....  | do.....       | (PVA<br>Gel) | Excellent.....<br>do..... | Excellent.....<br>Fair.....             | Excellent.....<br>NG..... |
| 4..... Tinopal TASC..... | do.....       | (PVA<br>Gel) | do.....                   | Excellent.....<br>NG.....               | Excellent.....<br>NG..... |
| 5..... Uvitex CF.....    | CIBA.....     | (PVA<br>Gel) | NG.....<br>NG.....        | Excellent.....<br>Good.....             | Excellent.....<br>NG..... |

NOTE.—NG indicates unsatisfactory stability, ft. cd., foot candles.

All of the above brighteners found to be unsatisfactory in gelatin are improved when used in polyvinyl alcohol.

Uvitex CF used in baryta formulations comparing gelatin versus polyvinyl alcohol binders for the baryta layer shows that it has significantly better stability to light, heat, and humidity in the polyvinyl alcohol baryta than in the gelatin baryta.

(1) Tinopal 4BM:



(2) Tinopal RBS: Sodium 4-(2H-naphtho[1,2-d]triazol-2-yl)-2-stilbenesulfonate:



(3) Tinopal AMS:



(4) Tinopal TASC:



(5) Uvitex CF:



Further addenda and variations in the compositions of the invention are discussed hereinafter.

The silver halide emulsions used in accordance with this invention can comprise silver chloride, silver bromide,

silver bromoiodide, silver chlorobromoiodide or mixtures thereof. The emulsions may be coarse or fine grain and can be prepared by any of the well-known procedures, e.g., single jet emulsions, double jet emulsions, such as Lippmann emulsions, ammoniacal emulsions, thiocyanate or thioether ripened emulsions such as those described in Nietz et al. U.S. Pat. 2,222,264; Illingsworth U.S. Pat. 3,320,069; and McBride U.S. Pat. 3,271,157. Surface

image emulsions may be used or internal image emulsions such as those described in Davey et al. U.S. Pat. 2,592,250; Porter et al. U.S. Pat. 3,206,313; Berriman U.S. Pat. 3,367,778 and Bacon et al. U.S. Pat. 3,447,927. If desired, mixtures of surface and internal image emulsions may be used as described in Luckey et al. U.S. Pat. 2,996,382. The emulsions may be regular grain emulsions such as the type described in Klein and Moisar, *J. Phot. Sci.*, vol. 12, No. 5, Sept./Oct. 1964, pp. 242-251.

The emulsions may be sensitized with chemical sensitizers, such as with reducing agents; sulfur, selenium or

tellurium compounds; gold, platinum or palladium compounds; or combinations of these. Suitable procedures are

described in Sheppard et al. U.S. Pat. 1,623,499; Waller et al. U.S. Pat. 2,399,083; McVeigh U.S. Pat. 3,297,447; and Dunn U.S. Pat. 3,297,446.



The emulsion can be protected against the production of fog and can be stabilized against loss of sensitivity during keeping. Suitable antifoggants and stabilizers each used alone or in combination include thiazolium salts

described in Brooker et al. U.S. Pat. 2,131,038 and Allen et al. U.S. Pat. 2,694,716; the azaindenes described in Piper U.S. Pat. 2,886,437 and Heimbach et al. U.S. Pat. 2,444,605; the mercury salts as described in Allen et al. U.S. Pat. 2,728,663; the urazoles described in Anderson et al. U.S. Pat. 3,287,135; the sulfocatechols described in Kennard et al. U.S. Pat. 3,236,652; the oximes described in Carroll et al. British Pat. 623,448; nitron; nitroindazoles; the mercaptotetrazoles described in Kendall et al. U.S. Pat. 2,403,927; Kennard et al. U.S. Pat. 3,266,897 and Luckey et al. U.S. Pat. 3,397,987; the polyvalent metal salts described in Jones U.S. Pat. 2,839,405; the palladium, platinum and gold salts described in Trivelli et al. U.S. Pat. 2,566,263 and Yutzy et al. U.S. Pat. 2,597,915.

The photographic and other hardenable layers used in the practice of this invention can be hardened by various organic or inorganic hardeners, alone or in combination, such as the aldehydes, and blocked aldehydes, ketones, carboxylic and carbonic acid derivatives, sulfonate esters, sulfonyl halides and vinyl sulfonyl ethers, active halogen compounds, epoxy compounds, aziridines, active olefins, isocyanates, carbodiimides, mixed function hardeners and polymeric hardeners such as oxidized polysaccharides, e.g., dialdehyde starch, oxyguargum and the like.

The photographic emulsions and elements can contain various colloids alone or in combination as vehicles, binding agents and various layers. Suitable hydrophilic materials include both naturally-occurring substances such as proteins, for example, gelatin, gelatin derivatives, cellulose derivatives, polysaccharides such as dextran, gum arabic and the like; and synthetic polymeric substances such as water soluble polyvinyl compounds like poly(vinylpyrrolidone), acrylamide polymers and the like.

The described photographic emulsion layers and other layers of a photographic element employed in the practice of this invention can also contain alone or in combination with hydrophilic, water permeable colloids, other synthetic polymeric compounds such as dispersed vinyl compounds such as in latex form and particularly those which increase the dimensional stability of the photographic materials. Suitable synthetic polymers include those described for example, in Nottorf U.S. Pat. 3,142,568, issued July 28, 1964; White U.S. Pat. 3,193,386, issued July 6, 1965; Houck et al. U.S. Pat. 3,062,674, issued Nov. 6, 1962; Houck et al. U.S. Pat. 3,220,844, issued Nov. 30, 1965; Ream et al. U.S. Pat. 3,287,289, issued Nov. 22, 1966; and Dykstra U.S. Pat. 3,411,911, issued Nov. 19, 1968; particularly effective are those water-insoluble polymers of alkyl acrylates and methacrylates, acrylic acid, sulfoalkyl acrylates or methacrylates, those which have cross-linking sites which facilitate hardening or curing and those having recurring sulfobetaine units as described in Dykstra Canadian Pat. 774,054.

The photographic elements used with this invention may contain antistatic or conducting layers; such layers may comprise soluble salts, e.g., chlorides, nitrates, etc., evaporated metal layers, ionic polymers such as those described in Minsk U.S. Pat. 2,861,056 and Sterman et al. U.S. Pat. 3,206,312 or insoluble inorganic salts such as those described in Trevoy U.S. Pat. 3,428,451.

The photographic layers and other layers of a photographic element employed as described herein can be coated on a wide variety of supports. Typical supports include cellulose nitrate film, cellulose ester film, poly(vinyl acetal) film, polystyrene film, poly(ethylene terephthalate) film, polycarbonate film and related films or resinous materials, as well as glass, paper, metal and the like. Typically, a flexible support is employed, especially a paper support, which can be partially acetylated or coated with baryta and/or an alpha-olefin polymer, particularly a polymer of an alpha-olefin containing 2 to 10 carbon atoms such as polyethylene, polypropylene, ethylenebutene copolymers and the like.

The photographic layers employed in the practice of this invention can contain plasticizers and lubricants such as polyalcohols, e.g., glycerin and diols of the type described in Milton et al. U.S. Pat. 2,960,404; fatty acids or esters such as those described in Robijns U.S. Pat. 2,588,765 and Duane U.S. Pat. 3,121,060; and silicone resins such as those described in Du Pont British Pat. 955,061.

The photographic layers employed in the practice of this invention may contain surfactants such as saponin, anionic compounds such as the alkyl aryl sulfonates described in Baldsiefen U.S. Pat. 2,600,831; amphoteric compounds such as those described in Ben-Ezra U.S. Pat. 3,133,816; and water soluble adducts of glycidol and an alkyl phenol such as those described in Olin Mathieson British Pat. 1,022,878.

The photographic elements employed in the practice of this invention may contain matting agents such as starch, titanium, dioxide, zinc oxide, silica, polymeric beads including beads of the type described in Jelley et al. U.S. Pat. 2,992,101 and Lynn U.S. Pat. 2,701,245.

The photographic elements used in this invention may contain brightening agents including stilbenes, triazines, oxazoles and coumarin brightening agents. Water soluble brightening agents may be used such as those described in Albers et al. German Pat. 972,067 and McFall et al. U.S. Pat. 2,933,390 or dispersions of brighteners may be used such as those described in Jansen German Pat. 1,150,274, Oetiker et al. U.S. Pat. 3,406,070 and Heidke French Pat. 1,530,244.

Spectral sensitizing dyes can be used conveniently to confer additional sensitivity to the light sensitive silver halide emulsion of the multilayer photographic elements which are developed in accordance with our invention. For instance, additional spectral sensitization can be obtained by treating the emulsion with a solution of a sensitizing dye in an organic solvent or the dye may be added in the form of a dispersion as described in Owens et al. British Pat. 1,154,781. For optimum results, the dye may either be added to the emulsion as a final step or at some earlier stage.

Sensitizing dyes useful in sensitizing such emulsions are described, for example, in Brooker et al. U.S. Pat. 2,526,632, issued Oct. 24, 1950; Sprague U.S. Pat. 2,503,776, issued Apr. 11, 1950; Brooker et al. U.S. Pat. 2,493,748; and Tabor et al. U.S. Pat. 3,384,486. Spectral sensitizers which can be used include the cyanines, merocyanines, complex (tri or tetrnuclear) merocyanines, complex (tri or tetrnuclear) cyanines, holopolar cyanines, styryls, hemicyanines (e.g., enamine hemicyanines), oxonols and hemioxonols.

The various layers, including the photographic layers, employed in the practice of this invention can contain light absorbing materials and filter dyes such as those described in Sawdrey U.S. Pat. 3,253,921; Gaspar U.S. Pat. 2,274,782; Silberstein et al. U.S. Pat. 2,527,583 and Van Campen U.S. Pat. 2,956,879. If desired, the dyes can be mordanted, for example, as described in Jones et al. U.S. Pat. 3,282,699.

The photographic layers used in the practice of this invention may be coated by various coating procedures including dip coating, air knife coating, curtain coating, or extrusion coating using hoppers of the type described in Beguin U.S. Pat. 2,681,294. If desired, two or more layers may be coated simultaneously by the procedures described in Russell U.S. Pat. 2,761,791 and Wynn British Pat. 837,095. This invention also can be used for silver halide layers coated by vacuum evaporation as described in British Pat. 968,453 and LuValle et al. U.S. Pat. 3,219,451.

This invention may be used with elements designed for colloid transfer processes such as described in Yutzy et al. U.S. Pat. 2,716,059; silver salt diffusion transfer processes such as described in Rott U.S. Pat. 2,352,014, Land 75 U.S. Pat. 2,543,181, Yackel et al. U.S. Pat. 3,020,155,

13

and Land U.S. Pat. 2,861,885; color image transfer processes such as described in Rogers U.S. Pats. 3,087,817; 3,185,567; and 2,983,606; Weyerts et al. U.S. Pat. 3,253,915; Whitmore et al. U.S. Pat. 3,227,550; Barr et al. U.S. Pat. 3,227,551; Whitmore U.S. Pat. 3,227,552; and Land U.S. Pats. 3,415,644; 3,415,645; 3,415,646; and imbibition transfer processes as described in Minsk U.S. Pat. 2,882,156.

This invention may be used with elements designed for color photography, for example, elements containing color-forming couplers such as those described in Frohlich et al. U.S. Pat. 2,376,679, Jelley et al. U.S. Pat. 2,322,027, Fierke et al. U.S. Pat. 2,801,171, Godowsky U.S. Pat. 2,698,794, Barr et al. U.S. Pat. 3,227,554 and Graham et al. U.S. Pat. 3,046,129; or elements to be developed in solutions containing color-forming couplers such as those described in Mannes et al. U.S. Pat. 2,252,718, Carroll et al. U.S. Pat. 2,592,243 and Schwan et al. U.S. Pat. 2,950,970; and in false-sensitized color materials such as those described in Hanson U.S. Pat. 2,763,549.

The invention has been described in detail with particular reference to preferred embodiments thereof, but it will be understood that variations and modifications can be effected within the spirit and scope of the invention.



I claim:

- An element comprising a support which has thereon a substantially protein-free layer containing barium sulfate, polyvinyl alcohol and an optical brightener, having 40 over said layer a layer of polyolefin.
- An element of claim 1 in which the support is paper.
- An element of claim 1 in which the polyolefin is polyethylene.
- An element according to claim 1 in which said layer contains a blue pigment.
- An element of claim 1 which contains in said layer about 3-15% by weight of said layer, of barium sulfate and about 0.02-0.50% by weight of said layer of optical brightener.
- An element of claim 1 in which said brightener is 50 water-soluble.



7. An element of claim 1, having over the said layer a receiving layer containing a silver precipitating agent.

14

8. An element of claim 1 having over the said polyolefin layer, a receiving layer comprising a silver precipitating agent.

9. An element of claim 1 having over said layer a light sensitive silver halide emulsion.

10. An element of claim 1 having over said polyolefin layer a light sensitive silver halide emulsion.

11. An element of claim 1 in which the optical brightener is a compound of the formula:



10 where R<sub>2</sub>, R<sub>3</sub>, R<sub>6</sub> and R<sub>7</sub> each represent a member selected from the group consisting of a hydrogen atom, a hydroxyl group, an aryloxy group, an alkoxy group, a halogen atom, a heterocyclic radical, an alkylthio group, an 15 arylothio group, and an amino group, and R<sub>4</sub> and R<sub>5</sub> each represent a member selected from the group consisting of a hydrogen atom, a sulfo group and a carboxyl group.

20 12. An element of claim 1 in which said brightener has the formula:



13. An element of claim 1 in which said brightener has the formula:



- Sodium 4-(2H-naphtho[1,2-d]triazol-2-yl)-2-stilbenesulfonate  
14. An element of claim 1 in which said brightener has the formula:



15. An element of claim 1 in which said brightener has the formula:



16. An element of claim 1 in which said brightener has the formula:



## References Cited

## UNITED STATES PATENTS

|           |        |                      |       |
|-----------|--------|----------------------|-------|
| 3,592,645 | 7/1971 | Weyerts et al. ----- | 96—82 |
| 3,269,840 | 8/1966 | Koerber et al. ----- | 96—82 |
| 3,512,984 | 5/1970 | Amano et al. -----   | 96—82 |

NORMAN G. TORCHIN, Primary Examiner

J. L. GOODROW, Assistant Examiner

U.S. CL. X.R.

96—76